

# UNITED STATES PATENT OFFICE.

ALEXANDRE ETIENNE LAVROFF, OF ST. PETERSBURG, RUSSIA.

## IMPROVEMENT IN ALLOYS OF COPPER AND TIN.

Specification forming part of Letters Patent No. 118,372, dated August 22, 1871.

*To all whom it may concern:*

Be it known that I, ALEXANDRE ETIENNE LAVROFF, of St. Petersburg, Russia, a colonel in the artillery guard, have invented Improvements in Compounds or Alloys of Copper and Tin, of which the following is a description:

My invention consists in an alloy or bronze, into the composition of which tin, copper, and phosphorus enter in definite proportions, viz., phosphorus, 1 per cent.; tin, 19 per cent.; copper, 80 per cent.

In compounding the alloy I first fuse the tin 19 per cent., or 94.5, and phosphorus 1 per cent., or 5.5.

This mass is added to the copper to form the

alloy in the following proportions: Mass—tin 94.5, phosphorus 5.5; copper, 400; which, otherwise stated, would be, about, phosphorus, 1; copper, 80; tin, 19.

The entire mass is then fused, and the alloy formed in the usual manner and ready for filling the mold.

Having thus described my invention, what I claim as new, and desire to secure by Letters Patent, is—

The alloy herein described.

ALEXANDRE ETIENNE LAVROFF.

Witnesses:

MICHEL SABLÉ,  
FREDERICK KAUFÉ.